

## UNITED STATES PATENT OFFICE

2,129,854

## MANUFACTURE OF LEATHER

Gustav Mauthe and Hermann Noerr, Leverkusen-I. G. Werk, Germany, assignors to I. G. Farbenindustrie Aktiengesellschaft, Frankfort-on-the-Main, Germany

No Drawing. Application November 21, 1935, Serial No. 50,989. In Germany November 28, 1934

9 Claims. (Cl. 149—5)

This invention relates to improvements in the manufacture of leather.

Minerally tanned leathers prepared with the aid of water soluble zirconium salts as tanning agents display some properties which impair their value. For example, after the usual rinsing, greasing and drying, they exhibit a rather hard feel. Although this is somewhat improved by subsequent staking, even then the finished leather still leaves much to be desired in this respect. A further disadvantage consists in the fact that the color of the finished zirconium-tanned leathers has a somewhat yellowish shade which can be noticed even if pure zirconium compounds have been employed and if the leathers have been greased with light-coloured water-soluble oils.

In accordance with our invention, these disadvantages can be diminished or practically 20 completely overcome.

The process of this invention comprises the step of acting on the leathers, during or after tanning, with non-tanning water soluble sulphonic or carboxylic acids containing aromatic nuclei or 25 water-soluble salts of such sulphonic or carboxylic acids. By the term "non-tanning", as used above and in the appended claims, such compounds are meant which, when used alone, are not capable of converting the animal skin into 30 leather. According to a further feature of our invention the said improvement becomes still more obvious if such aromatic compounds are used the molecular weight of which has been increased either by linkage of several nuclei or 35 by substitution, for instance, by hydroxyl groups or chlorine.

For instance, whereas the effect with benzoic acid is still rather small, the use even of dichlorobenzoic acid results in an evident improvement in 40 the leather quality as regards fullness and color. A similar good result is obtained by substituting into the molecule an aromatic nucleus, for instance a benzoyl residue. A considerable improvement can be attained by the application of 45 compounds containing hydroxyl groups such as chlorohydroxybenzoic acid. The aromatic dicarboxylic acids display a similar behaviour. Whereas, for example, the effect obtained by using phthalic acid is not yet sufficient for all practical purposes, dichloro- or tetrachlorophthalic acids prove themselves to be excellent auxiliary agents, as besides effecting an improvement in 50 color, softness, grain and resisting capacity towards hot water, they yield leathers which are absolutely fast to light. Here too the more com-

plicated compounds, for example those possessing two nuclei in the molecule, such as terephthalylbenzoic acid, display an outstanding effect.

With the sulphonic acids containing aromatic nuclei in a similar manner, the effect is dependent 5 on the constitution. The simple sulphonic acids of benzene and naphthalene show a relatively small, although noticeable efficacy, which results in a somewhat softer feel and an improvement in the fullness of the leather. A considerable increase of the efficacy is attained by replacing the simple sulphonic acids by, for example, substituted triphenylmethane sulphonic acids, such for instance as tetrachloro-dihydroxy-triphenylmethane sulphonic acids. 10

The treatment may be performed in various ways and at various stages of the tanning. It is possible, for instance, to employ the said compounds in the place of the usual neutralizing agents such as sodium bicarbonate; they may also be added to the tanning liquor subsequent to neutralization. A further possibility consists in the after-treatment of the tanned leathers in a fresh bath before or after the usual rinsing process. Even small amounts of the aromatic 25 compounds are sufficient, and they may be employed as such or in admixture with one another; on an average there is employed about 0.5 to 5% calculated on the weight of the hides. 15

In all cases the treatment results in an improved taking up of fat and an improvement in the quality of the leather as regards color, softness, fullness or feel. 30

The following examples illustrate the invention without limiting it thereto, the indications in 35 per cent being calculated on the weight of the hides:—

*Example 1*

Pickled calf hides are treated with an aqueous solution of sodium chloride and zirconium sulphate until they are well struck through. The leather thus prepared is treated for one to two hours in the drum with 100% of water and 5% of the sodium salt of naphthalene 1,5-disulphonic acid. The leather is then well rinsed, 45 greased, dried, stretched and staked. A white leather of improved fullness and outstanding fastness to light is obtained. 40

*Example 2*

Pickled calf hides are treated in accordance with the directions given in Example 1, the sodium salt of naphthalene 1,5-disulphonic acid being replaced by the same amount of the sodium salt of 2,2'-dihydroxy-3,5,3',5'-tetrachloro-tri- 55

phenylmethane - 2'' - sulphonic acid. By this treatment the softness and the whiteness of the leather are still more improved than by the treatment in accordance with the manner described in Example 1.

*Example 3*

Calf hide pickled with sulphuric acid is tanned with the employment of 8% of zirconium sulphate; after the hides are struck through, a pH-value of about 3 is established with the aid of sodium bicarbonate, whereupon the leather is drummed for two hours with 4% of dichlorophthalic acid in a fresh bath, kept in this bath over night, rinsed until a pH-value of 4.8 is attained, finally greased and dressed in the customary manner. The leather obtained exhibits an improved softness, white colour, dry feel and excellent fastness to light.

*Example 4*

A treatment is performed in accordance with the directions given in Example 3, replacing the dichlorophthalic acid by terephthalyl-2-benzoic acid. Fullness, softness, feel and the resisting capacity towards hot water are considerably improved in comparison with non-after-treated zirconium sulphate-tanned leathers; the fastness to light is scarcely less than that of the product prepared in the manner described in Example 3.

*Example 5*

A calf hide tanned with zirconium sulphate is after-treated with 5% of the sodium salt of 2,5-dichlorobenzoic acid in 100% of water, whereby, after rinsing, greasing and drying, an improvement in the fullness and softness of the leather is obtained.

*Example 6*

Instead of the sodium salt of dichlorobenzoic acid mentioned in Example 5 the sodium salt of 4'-chlorobenzoyl-2-benzoic acid can be employed with the same success.

*Example 7*

45 The dichlorobenzoic acid salt of Example 5 is replaced by the same amount of 5-chloro-2-hydroxybenzoic acid. Besides improved fullness, a finer white and a greater resisting capacity towards hot water is attained.

*Example 8*

A piece of goat hide which has been tanned with 8% of sodium sulphate and 2.5% of zirconium dioxide (as  $ZrOCl_2 \cdot 8H_2O$ ) in 100% of water is after-treated for two hours in a fresh bath to which 2% of a mixture of the sodium salts of the dichloro and tetrachlorophthalic acids are added. The hide is then thoroughly rinsed, greased with a light-coloured water-soluble oil and pole-dried. Whereas a hide which has not been treated in accordance with the process of this example and which has only been rinsed, greased and dried, shrinks very much and is hard after drying, the after-treated leather is much softer and fuller and possesses an excellent fastness to light.

*Example 9*

A goat hide tanned with zirconium oxychloride

is neutralized with sodium bicarbonate, stored for 24 hours, rinsed and after-treated with a solution of 2% of the sodium salt of tetrachlorophthalic acid. After rinsing, greasing and drying, similar differences can be observed in comparison with a non-after-treated leather to those pointed out in Example 8.

We claim:-

1. In the process of tanning with zirconium salts, the modification which comprises applying 10 to the leather, during or after tannage, a solution having incorporated therein a non-tanning compound containing an aromatic nucleus selected from the group consisting of watersoluble carboxylic and sulphonic acids and watersoluble 15 salts of carboxylic and sulphonic acids.

2. In the process of tanning with zirconium salts, the modification which comprises applying to the leather, during or after tannage, a solution having incorporated therein a non-tanning compound according to claim 1, in which compound the aromatic nucleus contains a substituent group. 20

3. In the process of tanning with zirconium salts, the modification which comprises applying to the leather, during or after tannage, a solution 25 having incorporated therein a non-tanning compound according to claim 1, which compound contains more than one aromatic nucleus.

4. In the process of tanning with zirconium salts, the modification which comprises applying 30 to the leather, during or after tannage, a solution having incorporated therein a non-tanning compound according to claim 1, which compound contains more than one aromatic nucleus and in which compound the aromatic nucleus contains a 35 substituent group.

5. In the process of tanning with zirconium salts, the modification which comprises applying 40 to the leather, during or after tannage, a solution having incorporated therein a non-tanning watersoluble halogenated aromatic acid, which may be present in the form of a watersoluble salt.

6. In the process of tanning with zirconium salts, the modification which comprises applying 45 to the leather, during or after tannage, a solution having incorporated therein a non-tanning watersoluble halogenated aromatic carboxylic acid, which may be present in the form of a watersoluble salt.

7. In the process of tanning with zirconium salts, the modification which comprises applying 50 to the leather, during or after tannage, a solution having incorporated therein a watersoluble salt of a chlorophthalic acid.

8. In the process of tanning with zirconium salts, the modification which comprises applying 55 to the leather, during or after tannage, a solution having incorporated therein a watersoluble salt of tetrachlorophthalic acid.

9. In the process of tanning with zirconium salts, the modification which comprises applying 60 to the leather, during or after tannage, a solution having incorporated therein a mixture containing alkali salts of di-, tri- and tetrachlorophthalic 65 acids.

GUSTAV MAUTHE.  
HERMANN NOERR.